

## UNITED STATES PATENT OFFICE

CYRIL J. STAUD AND ERIC K. MCLEAN, OF ROCHESTER, NEW YORK, ASSIGNORS TO EAST-MAN KODAK COMPANY, OF ROCHESTER, NEW YORK, A CORPORATION OF NEW YORK

PREPARATION OF LOWER MIXED ORGANIC ESTERS OF CELLULOSE FROM PARTIALLY HYDROLYZED CELLULOSE ACETATE

No Drawing.

Application filed October 3, 1931. Serial No. 566,794.

This invention relates to the preparation of cellulose esters of the nature of cellulose acetate-propionate by esterifying partially hydrolyzed cellulose acetate with an esterifying bath containing both the anhydride and the acid of the group, such as propionic, which is to be introduced into the cellulose molecule.

Heretofore it has been known to propionate or butyrate cellulose acetate by treating it in an esterifying bath containing propionyl chloride and pyridine. Propionyl chloride which is employed in that process is not readily available on a commercial scale and due to the expense involved, that process has not been carried out to a great extent on a commercial scale.

It has also been known to esterify cellulose acetate with a fatty acid anhydride and chloracetic acid, which is an excellent method of producing mixed esters of cellulose but that method has the disadvantage that chloracetic acid has a decidedly corrosive effect on the containing vessels in which it is employed.

We have now found a method of making cellulose acetate-propionates and cellulose acetate butyrates which is simple, rapid and easily controlled. We have found a method of making cellulose acetate-propionates which employs a partially deacetylated cellulose acetate such as for example commercially available acetone-soluble hydrolyzed cellulose acetate as the starting material, which is low in cost of materials and operation so as to be of commercial value and which is not corrosive of the equipment which is ordinarily employed for the esterification of cellulose.

We have found a method of making cellulose acetate-propionate or -butyrate which makes possible the dispersion of the partially esterified cellulose acetate prior to its esterification thus facilitating the esterification which may be carried out under conditions which are less severe than those which are ordinarily necessary to assure the proper esterification of cellulosic materials. We have found a method of making a cellulose acetate-propionate in which only a minimum of degradation, of any, takes place.

We have found that when a partially ester-

fied cellulose acetate having an acetyl content of about 35-38% is treated with an esterifying bath containing propionic acid, propionic anhydride and a catalyst, a cellulose acetate propionate is produced which is equal or even superior to the cellulose acetate-propionates heretofore produced. We have found that when the cellulose acetate is pretreated with the propionic acid, it may be dispersed in the acid, which condition is advantageous for the subsequent treatment with propionic anhydride and a catalyst.

The following example illustrates one method by which our invention may be carried out:

About 26 lbs. of a cellulose acetate having an acetyl content of about 36% is dissolved in 136 lbs. of propionic acid which is maintained at about 40°-50° C. for approximately 16 hours. The cellulose acetate is dispersed by this treatment. A mixture of 26 lbs. of propionic anhydride, 10 lbs. of propionic acid and .25 lbs. of magnesium perchlorate trihydrate is then added.

The mass is maintained between 50°-60° C. for about 5 hours. It may then be poured into water with vigorous stirring and the cellulose acetate-propionate will be precipitated out. This ester is soluble in ethylene chlorid, acetone, ethyl acetate, etc.

It is to be understood that our process may also be employed to produce cellulose acetate-butyrate, in which case equimolecular proportions of butyric acid and anhydride will be employed in place of the respective amounts of propionic acid and anhydride employed in our process.

The product of our process may be employed for film, filaments etc. from ethylene chloride, acetone or ethylene chloride-alcohol solutions of the same or if desired it may first be hydrolyzed according to the method disclosed in Malm and Fletcher application Serial No. 551,546 and the product resulting from that process may be employed to produce film or sheeting.

It is obvious that various modifications of our invention will be apparent to those familiar with the chemistry of cellulose esters

and all such modifications are within the contemplation of the present invention.

We claim as our invention:

1. A process of making a mixed ester of cellulose which comprises esterifying a partially hydrolyzed cellulose acetate with a reaction bath containing an acid and the corresponding anhydride each of which contains an acyl group selected from the group consisting of propionyl and butyryl.
2. A process of making cellulose acetate-propionate which comprises treating a partially hydrolyzed cellulose acetate with an esterifying bath containing propionic acid and anhydride.
3. A process of making cellulose acetate-propionate which comprises dispersing a partially hydrolyzed cellulose acetate in propionic acid and then esterifying the dispersed cellulose acetate in a reaction mixture containing propionic anhydride.
4. A process of making cellulose acetate-butyrate which comprises treating a partially hydrolyzed cellulose acetate with an esterifying bath containing butyric acid and anhydride.
5. A process of making cellulose acetate-butyrate which comprises dispersing a partially hydrolyzed cellulose acetate in butyric acid and then esterifying the dispersed cellulose acetate in a reaction mixture containing butyric anhydride.

Signed at Rochester, New York, this 24th day of September, 1931.

35 CYRIL J. STAUD.  
ERIC K. McLEAN.

40

45

50

55

60

65